

A. RIDD.

## PROCESS OF TREATING METAL SHEETS.

APPLICATION FILED JUNE 14, 1909.

961,462.

Patented June 14, 1910.

2 SHEETS—SHEET 1.



Witnesses

Witnesses  
F. J. Chapman.

Ambrose Ridd.

By *C. Brown Jr.*

Attorneys

A. RIDD.

PROCESS OF TREATING METAL SHEETS.

APPLICATION FILED JUNE 14, 1909.

961,462.

Patented June 14, 1910.

2 SHEETS—SHEET 2.



Witnesses

*F. T. Chapman*

By *Ambrose Ridd.*  
Attorneys

# UNITED STATES PATENT OFFICE.

AMBROSE RIDD, OF NEWPORT, KENTUCKY.

## PROCESS OF TREATING METAL SHEETS.

961,462.

Specification of Letters Patent. Patented June 14, 1910.

Application filed June 14, 1909. Serial No. 502,087.

*To all whom it may concern:*

Be it known that I, AMBROSE RIDD, a citizen of the United States, residing at Newport, in the county of Campbell and State 5 of Kentucky, have invented a new and useful Process of Treating Metal Sheets, of which the following is a specification.

This invention has reference to the process of treating metal sheets, and it is the 10 object of the present invention to insure uniformity of production so that the finished sheets shall be all alike.

In order that the present invention may be more clearly understood attention is 15 called to the usually employed method of treating metal sheets.

The sheets are first annealed in an air-tight box, or they are piled on a heavy slab, it being customary to treat from one hundred 20 to five hundred sheets at a time. If the slab be used then the sheets are charged into a muffle in bulk, that is, they are piled on the slab outside the furnace and are then introduced therein and the entire mass of 25 sheets is then annealed while lying flat on the slab. The temperature of the furnace is then lowered until a black heat is attained at which point the sheets are taken from the furnace in bulk and while still 30 resting on the said slab are carried in bulk to the rolls to be then fed sheet by sheet through the rolls, after which they are re-piled, on the opposite side of the rolls, on another heated slab and after all the sheets 35 have been rolled they are then charged into a furnace at a very low temperature and then allowed to cool off. Also when it is desired to oxidize certain of the sheets they are turned over singly while at a dark red 40 heat and are then taken to the rolls and finished as before except that the annealing is done in the regular air-tight box.

In accordance with the present invention the sheets are fed into the muffle chamber 45 singly and are then turned upon edge and when at the right temperature are turned down flat either singly or in packs. The sheets are then moved to the middle of the furnace and when at the right heat are 50 pushed out singly or in packs into an inclosed conduit, which is kept hot by super-heated steam or other non-oxidizing gas, from which conduit the sheets pass directly to the finishing rolls while still 55 bathed in a non-oxidizing gas. After passing through the finishing rolls the sheets

again enter a similar conduit at the opposite side of the rolls in which conduit the sheets cool off. For some purposes the conduit may be omitted and the sheets taken 60 directly from the furnace in full and free contact with the atmosphere and then passed through the rolls, or the rolling may be omitted.

The invention will be best understood 65 from a consideration of the following detail description taken in connection with the accompanying drawings forming a part of this specification in which drawings—

Figure 1 is a longitudinal vertical section 70 through a furnace constructed in accordance with the present invention. Fig. 2 is a section on the line A—B of Fig. 1. Fig. 3 is a longitudinal section of the discharge end of the furnace and the conduits leading to and 75 from the finishing rolls. Fig. 4 is a section on the line C—D of Fig. 3, more distant parts being omitted.

Considering first the apparatus used in the carrying out of the process herein disclosed, 80 which apparatus also forms a part of the present invention, there is shown a furnace 1, the showing being in part typical or diagrammatic since the structure shown is more illustrative than actual, although a furnace 85 constructed as shown will operate for the purposes of the present invention. It is not to be understood, however, that the showing of the drawings is at all mandatory since the furnace there shown and coöperating 90 parts may be greatly varied while still retaining the salient features of the invention.

Within the inclosing walls of the furnace and spaced therefrom so as to form a combustion space 2 there is a muffle chamber 3 95 accessible at one end through a series of doors 4. The floor 5 of the muffle chamber is shown as slanting, but of course this floor may be level if so desired. The openings closed by the doors 4 lead directly to the floor 100 5. Beneath this floor 5 are located furnaces 6 shown as three in number and extending laterally to the length of the muffle chamber, but this arrangement may also be varied as desired. It will be understood that the furnaces 6 lead to the combustion space 2 and that a suitable stack or chimney is connected to this combustion space for the escape of products of combustion after circulating well through the space 2 so as to thoroughly 110 and uniformly heat the muffle 3.

A pipe 7 leads into the muffle chamber 3.

and is there provided with a discharge nozzle 8 of any suitable type. The pipe 7 comes from a suitable source of supply of superheated steam, or in place of superheated steam any other suitable non-oxidizing gas may be conducted into the muffle through the pipe 7. The purpose of this pipe will appear further on.

The effect of superheated steam on a plate 10 at a cherry red heat is to produce a bluish coat or oxidation of the surface of the sheet, but such oxidation is so extremely thin as to have no practical value as a protective coating, therefore superheated steam may be defined as practically non-oxidizing.

At the end of the furnace remote from the doors 4 and opposite the middle door is an opening 9 and from this opening there leads a conduit 10 terminating at finishing rolls 20 11 and beyond these rolls is another conduit 12. Within the conduits 10-12 are rollers 13 forming supports for the sheets indicated at 14 on their way through the conduit 10 to the finishing rolls and through 25 the conduit 12 after leaving the finishing rolls. Adjacent to the opening 9 the conduit 10 carries feeding rollers 15 and extending through both conduits 10 and 12 are pipes 16 and 17 respectively having numerous perforations. These pipes are designed to carry superheated steam or hot air for a purpose which will presently appear.

In accordance with the method of treatment of the present invention the sheet 35 metal plates 14 are introduced into the muffle chamber 3 through the doors 4, usually the side doors, and are set on edge against the side walls of the muffle chamber, this permitting the sheets to be heated while 40 in a separated condition so that the sheets become heated uniformly throughout and are uniformly subjected to any oxidizing action which may take place. After the sheets have been properly heated they are 45 laid down flatwise on the bottom of the muffle chamber to form a pile which is moved to the middle point of the chamber in line with the conduit 10. Now the sheets are fed one at a time or in packs to the feed 50 rolls 15 and by the latter along the conduit 10 to the finishing rolls 11 and on leaving these latter into the conduit 12. During the heating of the sheets superheated steam or other non-oxidizing or practically non-oxidizing gas is introduced into the muffle chamber 55 through the pipe 7 so that the sheets are protected by the pressure thus established within the muffle chamber from the action of air entering through the openings normally closed by the doors 4 when the latter are opened for the purpose of handling the sheets and the edge discoloration so noticeable in sheets as heretofore treated is thereby avoided. Superheated 60 steam is introduced into the conduit 10 by

means of the pipe 16 and the temperature of the sheets 14 as they pass to the finishing rolls is thereby maintained. Steam is or may be introduced into the conduit 12 by means of the pipe 17. For oxidizing metal 70 sheets they are introduced into the furnace in the manner described and are brought to the required annealing temperature and then, if necessary, the temperature is gradually lowered while the sheets are still 75 within the muffle and when conditions are proper for exposing the plates the door is lifted and the plates or sheets are fed through the door singly until all have been discharged from the furnace. By this means 80 the sheets are uniformly heated and uniformly exposed to the oxidizing influence of the atmosphere and a uniform product is the result. When it is desirable to present the sheets to the finishing rolls then the sheets 85 within the muffle are kept bathed in an atmosphere of superheated steam or other non-oxidizing or practically non-oxidizing gas under sufficient pressure to prevent the entrance of atmospheric air to the muffle when 90 the doors are opened for the necessary handling of the sheets. Steam is caused to escape through the perforations in the pipe 16 and into the conduit 10 so that the sheets on their way from the muffle to the finishing 95 rolls 11 are bathed in a non-oxidizing atmosphere by means of which over-oxidation is prevented and the heat of the plates is maintained as they travel from the muffle to the rolls. After leaving the rolls the sheets pass 100 through the conduit 12 into which steam is introduced through the perforations in the pipe 17 and the sheets are thereby bathed in a non-oxidizing atmosphere but which is so regulated as to permit the sheets to cool 105 down so that when they reach the atmospheric air they are cooled sufficiently to be no longer oxidized thereby and the annealing to which these sheets have been subjected is then not affected by the cold atmosphere. 110

It is to be noted that the muffle chamber is rendered proof against the introduction of cold atmospheric air on the opening of the doors for the purpose of introducing sheets 115 to be annealed or for the purpose of withdrawing such sheets from the muffle chamber, by the introduction of a non-oxidizing gas at sufficient pressure to prevent the entrance into the muffle chamber of the atmospheric air when the muffle is opened. Hot air may be introduced with the superheated steam and since superheated steam is practically non-oxidizing the mixture of superheated steam and hot air may be made to 125 produce any degree of oxidation desired.

The present process forming the subject matter of this invention has marked advantages over prior processes in that there results a uniformity of color because each 130

sheet is exposed to the oxidizing influence of the air while all the sheets are at the same temperature, the color and oxidation resulting being therefore uniform. Furthermore, discoloring and overoxidation of the edges of the sheets, which has hitherto been unavoidable is completely overcome by the present process.

It will be understood that the furnace shown and described may be used for and is specially adapted to the heating of metal sheets that are to receive the Russia finish either by the ordinary hammering process or by the loose rolling or the friction rolling processes. The furnace disclosed is not herein claimed, but this is not to be construed as a waiver of the right to make subsequent application for Letters Patent therefor.

What is claimed is:

10. 1. The process of treating metal sheets consisting in heating the metal sheets, while on edge and in separated relation one to the other, in a bath of practically non-oxidizing gas, and then withdrawing said sheets one 15 by one from the heating zone while maintaining them in a bath of non-oxidizing gas.

20. 2. The process of treating metal sheets consisting in heating the metal sheets in a muffle chamber in a bath of practically non-oxidizing gas at super-atmospheric pressure while said sheets are on edge, and then withdrawing said sheets from the muffle chamber one at a time while maintaining the supply 25 of said gas in the muffle chamber.

30. 3. The process of treating metal sheets consisting in heating the metal sheets on edge in a muffle chamber in a bath of practically non-oxidizing gas at super-atmospheric pressure, then laying said sheets flat- 35 wise one upon another to form a stack, and

then withdrawing said sheets one at a time while maintaining the supply of said gas in the muffle chamber.

4. The process of treating metal sheets consisting in heating the metal sheets in a muffle chamber in a bath of practically non-oxidizing gas at super-atmospheric pressure and then feeding the sheets to finishing rolls through a bath of hot non-oxidizing gas exterior to the muffle chamber to prevent overoxidation of the sheets and to maintain their temperature as they pass to the rolls. 45

5. The process of treating metal sheets consisting in heating the sheets in a muffle chamber in the presence of practically non-oxidizing gas at super-atmospheric pressure, then passing the sheets from the muffle chamber to the finishing rolls through hot non-oxidizing gas, and then cooling the sheets after passing the finishing rolls in an atmosphere of non-oxidizing gas. 55

6. The process of treating metal sheets consisting in heating the sheets while on edge in a muffle chamber in the presence of practically non-oxidizing gas at super-atmospheric pressure, then laying the sheets flatwise one upon the other, then moving the sheets one at a time out of the muffle chamber to finishing rolls and maintaining about the sheets an atmosphere of hot non-oxidizing gas, and finally permitting the sheets to cool after passing the finishing rolls in an atmosphere of non-oxidizing gas. 65

In testimony that I claim the foregoing as my own, I have hereto affixed my signature in the presence of two witnesses.

AMBROSE RIDD.

Witnesses:

JNO. C. DE MOSS.  
JOHN MOSPENS.